

Dec. 22, 1953

G. A. ESPERSEN

2,663,069

METHOD OF MAKING INCANDESCENT CATHODES

Filed July 20, 1951



*Fig. 1.*



*Fig. 2.*

INVENTOR.  
GEORGE A. ESPERSEN.

BY 

AGENT.

## UNITED STATES PATENT OFFICE

2,663,069

METHOD OF MAKING INCANDESCENT  
CATHODESGeorge A. Espersen, Dobbs Ferry, N. Y., assignor  
to Philips Laboratories, Inc., Irvington-on-  
Hudson, N. Y.

Application July 20, 1951, Serial No. 237,695

9 Claims. (Cl. 29—25.14)

1

My invention relates to the manufacture of incandescent cathodes of the dispenser type which have a porous wall portion of refractory material.

The invention is particularly useful in connection with cathodes of the general type described in U. S. Patent 2,543,728 to H. J. Lemmens et al. and will be described in this connection. However, the invention is suitable to other types of cathodes where it is essential to make a tight joint between a porous member of refractory metal and a second member of refractory metal which members form a cavity containing an electron emissive material.

Cathodes described in the above-mentioned patent comprise a structure enclosing a cavity containing a supply of electron emissive material which structure has a porous wall portion of sintered refractory material, such as tungsten, which forms the emissive part of the cathode. As the pores of this porous portion must form the largest passageways connecting the cavity to the outside of the cathode and as such pores are of extremely small size, it is essential that a very tight joint be made between the porous portion and the remaining part of the cathode structure.

The main object of my invention is to produce a tight joint in such cathode structures.

A further object is to provide a simple and inexpensive method of producing such a joint.

A still further object is to produce a joint which remains tight during the operation of the cathode and may even increase in tightness with increasing operating temperatures.

Another object is to produce a tight joint without deleteriously affecting the electron emissive material present in the cavity.

In accordance with the method of my invention, I form the porous body by pressing into the desired shape a mass of particles of refractory metal, such as tungsten and then heat the so-formed body at a temperature which is sufficiently high to give the body good mechanical strength. This body, which will be referred to as the presintered body, will usually be sufficiently accurately dimensioned so as to fit with a snug fit, the body with which the tight joint is to be made. However, in some cases I prefer to machine the surface of the porous body so as to obtain the desired snug fit. For this purpose I may use the method disclosed in U. S. patent application S. N. 234,513, filed June 30, 1951 by Roberto Levi.

The presintered porous body is then slipped over the second body which has a higher volu-

2

metric coefficient of expansion than the refractory material to form a cathode assembly having a cavity in which the electron emissive material is provided. The cathode assembly is then heated at a temperature higher than the first temperature to produce a shrinking action in the porous body and a tight shrunken joint, because the second body will expand to a greater extent than the refractory material.

10 The temperatures to be used depend upon several factors including the refractory material used, the size of the particles and the pressures used. In the presintering I use a temperature which gives the body good mechanical strength and at the same time is considerably below that temperature to be used in the second heating operation. The temperature used during the second heating operation should be below that temperature at which the electron-emissive material would be deleteriously affected i. e. below its melting point, and at the same time should be sufficiently above the temperature first used to produce the necessary degree of shrinkage action and thus a tight seal. Care must, of course, be taken that the temperature used during the second operation is not so high as to produce an excessive shrinkage action which might tend to crack the porous body.

I have found that when using a porous tungsten body which is to be jointed to a molybdenum body good results have been obtained when using a temperature of about 900—1000° C. for the presintering operation and a temperature between about 1300° C. and 1800° C. for the sintering or shrinkage operation. However, as stated, the exact temperatures to be used will vary depending upon several factors and one skilled in this art can readily select the same.

40 To prevent undesired evaporation of the electron emissive material, I prefer to carry out the heating of the cathode assembly in an inert atmosphere, such as helium or argon, or in a slightly reducing atmosphere, such as nitrogen containing a few percent of hydrogen.

In order that my invention may be clearly 45 understood and readily carried into effect, I shall describe the same in more detail with reference to the accompanying drawing in which:

Figure 1 is a sectional side view on an enlarged scale of a dispenser type cathode of the cylindrical type, and

Figure 2 is a sectionized side view of a dispenser type cathode of the end emissive type.

The cathode shown in Figure 1, which is particularly useful in magnetrons, comprises a tubular member 1 of refractory metal, for instance

molybdenum, provided with a groove 2 containing a supply of electron emissive material 3, such as barium and strontium carbonates. Fitting upon the member 1 with a shrunken fit is a porous tubular body 4 of sintered refractory material, such as tungsten. A heating filament 5 is located within the bore of member 1.

In accordance with the method of the present invention the body 4 is made by pressing, for instance under a pressure of about 2,000 kg./cm.<sup>2</sup> a mass of finely-divided refractory metal such as tungsten in the desired form and for this purpose I make use of tungsten powder having a density of 54 gms./in.<sup>3</sup> and comprising the following fractions in the following proportions as determined by the elutriation test:

| Fraction | Radius                | Proportion by Weight, Percent |
|----------|-----------------------|-------------------------------|
| I.       | Over 6.1 $\mu$        | 30.9                          |
| II.      | Between 6.1-3.6 $\mu$ | 30.6                          |
| III.     | Between 3.6-2.9 $\mu$ | 13.3                          |
| IV.      | Between 2.9-2.2 $\mu$ | 7.6                           |
| V.       | Between 2.2-1.5 $\mu$ | 17.6                          |

The presintered body 4 is then slipped over member 1 with the electron emissive material 3 present in the cavity so as to give the cathode structure shown in Figure 1.

The assembled cathode structure is then heated in an inert atmosphere such as helium or nitrogen to sinter body 4 with a minimum amount of reduction of alkaline earth compound and thereby impart a shrinking action thereto so that body 4 embraces member 1 with a shrunken fit. For this purpose I heat the cathode structure to a temperature which is considerably above the temperature used in the presintering, for instance about 200° C. to 400° C. higher. On the other hand the temperature must be below that value at which the electron emissive material would be deleteriously affected. In general, I have found that when using tungsten, temperatures between about 1400° C. and 1800° C. are satisfactory.

The cathode shown in Figure 2, which is of the end-emitting type comprises a tubular body 6 provided with a partition 7 dividing the bore thereof into two parts. Fitting over the end of body 6 with a shrunken fit is a cup-shaped porous member 8 of refractory metal, such as tungsten. Member 8 forms with the upper portion of body 6 a cavity in which is located a supply 3 of electron emissive material such as barium and strontium carbonates. A heating filament 5 is located in the lower part of the body 6.

The cup-shaped body 8 is made in a manner similar to that disclosed in connection with body 4 and after being assembled into the cathode structure, the entire assembly is heated in the manner described in connection with Figure 1.

While I have described my invention in connection with specific examples and certain temperatures, pressures and particle sizes, I do not desire to be limited thereto as obvious modifications will readily present themselves to one skilled in this art.

What I claim is:

1. A method of manufacturing a cathode of the dispenser type comprising the steps of forming particles of a refractory metal under pressure into a hollow body open at one end thereof, presintering the so-formed body at a temperature high enough to impart sufficient mechanical strength thereto to make said body

self-supporting, forming a second body of a material having a higher volumetric coefficient of expansion than the refractory metal, said second body having a shape adapted to fit into the open end of said first body and forming an internal cavity therewith for containing a supply of alkaline earth metal compound, inserting said second body into said first body, and heating said first and second bodies to a temperature higher than the temperature at which said first body was presintered to tightly close the internal cavity by internally expanding the second body to a greater extent than the first body.

2. A method of manufacturing a cathode of the dispenser type comprising the steps of forming particles of tungsten under pressure into a hollow body open at one end thereof, presintering the so-formed body at a temperature high enough to impart sufficient mechanical strength thereto to make said body self-supporting, forming a second body of a material having a higher volumetric coefficient of expansion than the tungsten, said second body having a shape adapted to fit into the open end of said first body and forming an internal cavity therewith for containing a supply of alkaline earth metal compound, inserting said second body into said first body, and heating said first and second bodies to a temperature higher than the temperature at which said first body was presintered to tightly close the internal cavity by internally expanding the second body to a greater extent than the first body.

3. A method of manufacturing a cathode of the dispenser type comprising the steps of forming particles of tungsten under pressure into a hollow body open at one end thereof, presintering the so-formed body at a temperature high enough to impart sufficient mechanical strength thereto to make said body self-supporting, forming a second body of molybdenum, said second body having a shape adapted to fit into the open end of said first body and forming an internal cavity therewith for containing a supply of alkaline earth metal compound, inserting said second body into said first body, and heating said first body and second bodies to a temperature higher than the temperature at which said first body was presintered to tightly close the internal cavity by internally expanding the second body to a greater extent than the first body.

4. A method of manufacturing a cathode of the dispenser type comprising the steps of forming particles of tungsten under pressure into a hollow body open at one end thereof, presintering the so-formed body at a temperature high enough to impart sufficient mechanical strength thereto to make said body self-supporting, forming a second body of molybdenum, said second body having a shape adapted to fit into the open end of said first body and forming an internal cavity therewith for containing a supply of alkaline earth metal compound, inserting said second body into said first body, and heating said first and second bodies to a temperature higher than the temperature at which said first body was presintered to tightly close the internal cavity by internally expanding the second body to a greater extent than the first body.

5. A method of manufacturing a cathode of the dispenser type comprising the steps of forming particles of tungsten under pressure into a hollow body open at one end thereof presintering the so-formed body at a temperature of about 900° to

1000° C. to impart sufficient mechanical strength thereto to make said body self-supporting, forming a second body of molybdenum, said second body having a shape adapted to fit into the open end of said first body and forming an internal cavity therewith for containing a supply of alkaline earth metal compound, inserting said second body into said first body, and heating said first and second bodies to a temperature of about 1300° to 1800° C. to tightly close the internal cavity by internally expanding the second body to a greater extent than the first body.

6. A method of manufacturing a cathode of the dispenser type comprising the steps of forming particles of tungsten under pressure of about 2000 kg./cm.<sup>2</sup> into a body open at one end thereof, presintering the so-formed body at a temperature of about 900° to 1000° C., forming a second body of molybdenum, said second body having a shape adapted to fit into the open end of said first body and forming an internal cavity therewith for containing a supply of alkaline earth metal compound, inserting said second body into said first body, and heating said first and second bodies to a temperature of about 1300° to 1800° C. to tightly close the internal cavity by internally expanding the second body to a greater extent than the first body.

7. A method of manufacturing a cathode of the dispenser type comprising the steps of forming particles of tungsten into a hollow body open at one end thereof, presintering the so-formed body at a temperature of about 900° to 1000° C., forming a second body of molybdenum, said second body having a shape adapted to fit into the open end of said first body and forming an internal cavity therewith for containing a supply of alkaline earth metal compound, inserting said second body into said first body, and heating said first and second bodies to a temperature of about 1300° to 1800° C. in a non-oxidizing atmosphere to tightly close the internal cavity by internally expanding the second body to a greater extent than the first body.

8. A method of manufacturing a cathode of the dispenser type comprising the steps of forming particles of tungsten under pressure into a hollow body open at one end thereof, presintering the so-formed body at a temperature of about 900° to 1000° C. in a non-oxidizing atmosphere forming a second body of molybdenum, said second body having a shape adapted to fit into the open end of said first body and forming an internal cavity therewith for containing a supply of alkaline earth metal compound, inserting said second body into said first body, and heating said first and second bodies to a temperature of about 1300° to 1800° C. in a non-oxidizing atmosphere to tightly close the internal cavity by internally expanding the second body to a greater extent than the first body.

9. A method of manufacturing a cathode of the dispenser type comprising the steps of forming particles of tungsten under pressure into a hollow body open at one end thereof, presintering the so-formed body at a temperature of about 900° to 1000° C. to impart mechanical strength thereto, forming a second body of molybdenum, said second body having a shape adapted to fit into the open end of said first body and forming an internal cavity therewith for containing a supply of alkaline earth metal compound, inserting said second body into said first body, and heating said first and second bodies to a temperature of about 1300° to 1800° C. in hydrogen to tightly close the internal cavity by internally expanding the second body to a greater extent than the first body.

GEORGE A. ESPERSEN.

References Cited in the file of this patent

UNITED STATES PATENTS

| Number    | Name            | Date          |
|-----------|-----------------|---------------|
| 1,766,865 | Williams et al. | June 24, 1930 |